

## UNITED STATES PATENT OFFICE.

JOHN S. NOWOTNY, OF CINCINNATI, OHIO.

## ELECTRICAL RESISTANCE MATERIAL.

No Drawing.

Application filed June 13, 1921. Serial No. 477,265.

*To all whom it may concern:*

Be it known that I, JOHN S. NOWOTNY, a citizen of the United States, and residing at Cincinnati, in the county of Hamilton and State of Ohio, have invented a new and useful Improvement in Electrical Resistance Material, of which the following specification is a full disclosure.

This invention relates to the discovery of certain new and unique electrical property materials and to the process of making. The principal object of the invention or discovery is to produce a composite material having a predetermined and definite electrical property, such as resistance or conductivity.

Another object of the invention is to produce such a material of a nature adapting it to fabrication by molding or pressing or otherwise working into the shapes desired, adapting the material to be constituted into any suitable electrical apparatus element.

That is to say, a property of this material is that it can be fabricated either under cold or heat processes, as a dry, plastic or molten mass, depending upon the particular electrical apparatus element required.

In consequence, the element so formed from my new material may be given any desired mechanical strength, size of element, cubic or area dimension, having a predetermined thermal electric current conductivity or resistivity and which will also be a durable and staple article, the predetermined electrical property being constant and not subject to the usual variations such as increasing resistance under repeated heatings.

I have discovered that various materials or substances of relatively varying electrical property, each of which is capable of reduction by crushing, grinding or attrition into a granular or powdered mass, can be mixed or combined into a substantially homogeneous solid body, which body also is characterized by being relatively non-ductile, capable of being reduced by attrition.

The required electrical property can be definitely predetermined and controlled and rendered constant by the selection of and the relative proportions of the series of components, each of which has a different coefficient of the desired electrical property as instance by resistance.

Example, to construct a resistance element of high percentage, resistance materials of low conductivity are employed, and for an element of low percentage resistance, materials of high conductivity are used.

It is a characteristic of my newly discovered material that a given compound, that is, a given selection of material of different electrical properties combined in a given proportion through a wet process whereby a plastic mass is molded into shape and dried, possesses a different degree of resistivity, than the same kind and proportion of materials when fabricated by ceramic processes.

The discovery is clearly distinguishable from materials formed with metallic components. My product not only offers a very much wider range of selectivity but is definitely controllable as to the coefficient of electrical property, which coefficient remains constant.

Metallic resistance material is usually of low resistivity, while if refractory metal or compounds are used, which may have a high specific resistance to be used on high voltages, such materials are generally fragile and cannot be molten under commercially variable temperatures so as to be molded or cast into the desired shapes. Such materials, having vitreous properties, are undesirable heater elements and materials which I have discovered and constituted are relatively non-vitreous.

As illustrating fields of usage for my material they are generally adapted to constitute any desired electrical apparatus element such as heating devices, rheostats for controlling currents or fields of electrical generators, starting boxes for graduating the flow of electric current through motor armatures, or for controlling or regulating the speed of motor armatures for continuous service.

These materials can be made to stand very high temperatures without disintegration, fusing, or deterioration in electrical property, and the difference in coefficient remains very slight within a wide range of changes of temperatures, or, in other words, there is substantial constancy.

In general, the several materials of different electrical property, say for instance, iron oxide, lime and carbon are reduced to

a granular or powdered state and blended and combined in proportions determined by the desired electrical property.

When it is desired to produce an electrical resistance material of high percentage, the product is composed of certain proportions of these materials of low conductivity. For medium or low resistance, a lesser amount or proportion of the low conductive materials and a greater amount or proportion of relatively high conductivity materials are employed. Thus it is that both the selection and proportion of materials constitute the controlling agency for obtaining the predesired electrical property which predesired electrical property is variable and dependent upon this selection and proportion.

The compound may be pressed into shape and the resistance capacity gauged by the degrees of pressure delivered in shaping. If the press is employed with a gauge device, indicating the pressure in pounds applied, and the press dies or molds equipped or in connection with electrical measuring instrument, as an ohm-meter, the mass can be pressed into as compact a body as may be desired and the ohmic resistance accurately determined while the body is being formed.

Under a ceramic treatment or process the blended or conglomerate electrical resistance material may be combined with a bonding material, preferably of neutral character in a dry, semi-dry or liquid form and conditioned to make it workable for forming into the desired shapes under hydraulic or mechanical press pressures. The shaping of the resistance bodies can also be carried out by any of the well-known methods of uniting plastic materials. For curing, the bodies are then dried and placed in a suitable kiln or electric furnace. The temperature of the kiln may be raised sufficiently to thoroughly bond the materials or raised up to or beyond a firing point in order to eliminate or expel any foreign matter that may afterward be detrimental to the use of the composite under extraordinary temperatures, such as electric heating devices, or any beyond those employing ordinary temperatures, such as motor starters and controls and generator field controls. The heating or firing temperatures regulate the internal resistance of the body and a variation is produced by high or low temperatures.

The composite, as a body, may be heated by passing an electric current of sufficient amperage therethrough, so as to cause an intense heating of the composite and thereby bring the molecular parts, having an affinity for each other, into close or intimate contact with each other by thermo-union or electric welding. That is, the constituted material is preferably cured and so rendered staple and constant as to electrical property.

After such electric treatment, the body

may be again reduced by crushing and grinding, and the crushed material utilized as an article of commerce, for making resistance bodies, either by pressing, plastic molding or forming in a molten state. Conductor connections can be made by fractionally clamping, or by brazing or fusing the parts together.

In the light of this disclosure, it will be evident that the range of materials available, is quite extensive, and in giving examples, it is the purpose of stating them by way of illustration, and not as limiting the scope of the invention.

Also, it is my object to give examples with which I have obtained best results, and also to give due consideration to the cheapness and commercial availability of materials.

In general, the materials may be understood as embracing a combination of relatively high, medium, and low resistance material, lending itself to the arbitrary formula H M L. As an example of high resistance component, I have obtained the best results from the use of hydraulic cement, or any like material which will harden in water, oxide of calcium mixed with fire-clay, or the like, constituting the H formula element. As an example of the medium resistance component, best results have been obtained from the use of iron or tungsten oxide, or the like, which will be the M component of the formula. For the low resistance element, I preferably employ graphite, or coke, thus deriving the formula H M L. These materials are each reduced to a fine powder, and thoroughly mixed and blended for treatment in an electric furnace, preferably of the type in which the treatment charge is subjected to an electric current. As a proportional example, say I use 55% H, 40% M and 5% L, bringing it to a molten state, and adding, if desired, additional L to compensate for the loss of carbon by oxidation.

The treated material is taken from the furnace as an ingot, and it is a unitary body, in the nature of an alloy, having substantially homogeneous molecular electrical resistance, of say 1000 ohms per unit mass. This ingot product is suitable, say for a field control element and can be cast into the desired shape and structure. Or, the ingot material can be ground into a powder and by ceramic process pressed into a suitable electrical apparatus element structure.

But, if I desire say a heating element, the ingot body having too great a resistance, is itself taken as the H element, for an additional ceramic treatment. That is, the ingot is reduced to an H powder and again molded or blended with the M and L elements.

To indicate the lesser resistance property of the ingot material in relation to the original high resistance material, it may be des-

ignated as H- for the formula H-, M, L, to be constituted for the ceramic treatment producing a heating element.

Say I desire a heating element of approximately 5 ohms resistance per unit mass, I 5 powder, mix and blend say 60% H- 30% M and 10% L, preferably in a wet state, using water, silicate of soda, molasses, coal tar, or the like as a bonding agency. This 10 plastic mass is placed in a suitable (hydraulic) press and pressed into a shape or size corresponding to the structural nature of the desired element. The specific gravity, as well as the ohm resistance, per unit mass, 15 will depend somewhat upon the degree of pressure, which is, of course, controllable, and I recommend say a pressure of 2000 pounds to the square inch.

The element so formed is a brick-like body, 20 having a uniform and substantially constant resistance, it is non-ductile, reducible by attrition, substantially non-vitreous and physically entirely suitable to its usage, as well as having the predesired electrical properties. Moreover, it may be given any desired specific gravity, area or cubic dimensions, as well as structure desired.

It will, therefore, be readily understood, 25 and the importance of the fact observed, that by the selection and proportion, of the H M L elements in the first instance, or the H- M L elements in the second instance, and the pressure being a controllable agency, that I can, within a practical degree controllably predetermine not only the coefficient 30 of ohm resistance per unit mass, but the specific gravity, size, shape, structure and cubic or area dimension—i. e. shape and area of radiating surface of the heating element depending upon its condition of usage 35 or the apparatus requirement.

As another example, if the proportions for the ceramic treatment be, say 50% H- 30% M and 20% L, the product would be 40 substantially 3 ohm resistance per unit mass with a given pressure.

Or, 30% H- 50% M- and 20% L, would give a product, say, having a 2 ohm resistance per unit mass with the given degree of 45 pressure.

In constituting the primary or ingot material, say it be known or determined that the ohm resistance of the H is 10000, of the M 1000, and of the L 5, the ohm resistance 50 of the resultant product will depend upon the proportions, and this has to be determined and tabulated.

The same is true of the ceramic formula H- M L. Without attempting the infinite 55 proportional elaboration possible, the few examples selected will suffice to furnish a key enabling the discovery to be operated and in terms of formula, with a reasonable degree of accuracy and obtaining any desired coefficient of resistivity or conductiv-

ity. That is to say, if the given 3 different proportions of the H- M L bodies be made, their ohm resistance per unit mass, and with a given pressure, and their specific gravity determined, the results can be tabulated, as 70 for example:

60% H-30% M, 10% L= 5 ohm per unit mass.

50% H-30% M, 20% L= 75 5 ohm per unit mass.

30% H-50% M, 20% L= 2 ohm per unit mass.

The proportions can be infinitely varied, 80 and a working table so compiled from the determined data, enabling a most elastic and selective range of values to be obtained suitable to the requirements of a given usage or an arbitrary requirement if desired for any particular purpose. 85

It will thus be seen that the exact substance and proportions are not of limiting import inasmuch as this disclosure constitutes an entirely practicable, controllable and workable basis for obtaining the desired materials or products. 90

Series A—If it be desired to produce a material, say about 1000 ohm resistance per cubic centimeter, which may be relatively regarded as a high resistance material— 95

A—Formula—H. 50%  
M. 40%  
L. 10%

mould into shape under a pressure of approximately 4000 lbs., then heat to a temperature of about 750 F.—400 C. in enclosed sager or retort for a period of about 48 hours. 100

Series B—If it be desired to produce a material having 500 ohms resistance per cubic centimeter—take formula H. M. L. as indicated by A—; reheat to a temperature of say 2000 F.—1300 C. which will reduce A to B or 50% of its former internal resistance in ohms. 110

Series C—To produce a lower resistance material say 100 ohms to a cubic centimeter—

Take a formula H. 10%  
M. 40%  
L. 50%

Before or after having been pressed into shape and thoroughly dried, place in enclosed sager or retort and heat for about 48 hours, at a temperature of near 750 F.—400 C. 120

Series D—If still lower resistance is desired, say 50 ohms per cubic centimeter, after C mass or unit has been allowed to cool, re-bake formula C mass or unit for about 48 hours at a temperature of near 1500 F.—820 C. This will reduce C to D. 125

Series E—The resistance may again be lowered say to one ohm per cubic centimeter 130

by again bringing the temperature up to about 2000 to 2400 F.—1095 to 1300 C. either at a first, second or third baking as may be desired. This will change the resistance of 5 D to E unit.

That is to say a greater proportion or percentage of L— in relation to M and H— will decrease the ohms resistance, or a greater proportion of H or M— will proportionally increase the resistance.

Or increased pressure in forming into shape will decrease the resistance— or an increased temperature short of the destructive point in the baking or heating will more 15 thoroughly flux and consequently bring the molecular parts into closer contact, hence will decrease the resistance of the alloy so formed.

It may be fully understood that anyone 20 skilled in the art and being provided with the various formulas and a key to them, can readily produce commercially in any quantity, a resistance material that will fully meet all the requirements of the trade, from 25 the lowest say .50 ohms to 50,000 or more or less ohms per cubic centimeter, as may be required and predetermined by and at the will of the operator manufacturing various 30 formulas. The materials used to make H. M. L. formulas may be blended in their proper proportions and then heated to whatever 35 temperature needed to get the desired resistance of the mass or ingot without having been shaped. This mass of material can then be taken from furnace, retort or sager and crushed and ground and can be employed at any later time for the forming into resistance units of any required resistance by proportioning the various H. 40 M. L. mixes or formulas. This ground H. M. L. material may be packed and shipped in bulk, as H. formula numbered, M. formula numbered and L. formula numbered, for the use of manufacturers of resistance 45 appliances, and can be formed into any desired shape or predetermined resistance to suit the requirements—then heated or baked to finish product for use.

It can readily be observed that by employing 50 the H. M. L. series of varying resistance material, I can easily balance my proportions and predetermine the exact resistance of unit, mass or individual element alloy in process of formation. A slight addition of 55 H. and a small reduction of L., would cause increased resistance, or a slight addition of L. and a small reduction of H., would cause a reduction of resistance— or more or less of M. added to H. or L. would change the resistance in either a high or low direction, the percentage in the amounts of H. M. L., would be followed automatically by an increased or decreased ohms resistance in the finished product so formed.

60 To produce an L. mass of very low resist-

ance for blending with H. or M.—a very desirable formula which I indicate as formula F. in which I employ proportions viz—

H—20% by weight.  
M—60% by weight.  
L—20% by weight.

70

After the proportions of formula F. have been thoroughly mixed or blended, the entire mass before being moulded into shape 75 is placed in retort or furnace and heated to a temperature of about 1800 F.—985 C. While being fused in retort or sager the free circulation of air is excluded, that is to say, the retort is sealed to create a semi- 80 vacuum, the heat pressure in the retort preventing the outer air from entering freely into retort, of course the gas liberated from M is consumed, but the tendency of combustion or the complete oxidization of the 85 mass is thereby prevented, while the mass is being formed, which is known as formula F. L.

This mass is taken out of retort and 90 crushed and ground for future use in making up finished products, by being incorporated with H. and M. The H. and M. formulas can also be prepared in simliar manner to F. L., but it may be stated that various 95 temperatures are employed in the forming process.

While I have disclosed this general H. M. L. formula, as the best means of explaining the usage of this discovery, I do not mean to be understood as limiting the invention to 100 a material necessarily limited to three components only. For instance, it may be desirable to embrace in the H. unit, several species, such as a cement or fire-clay, or in the M. unit, say both manganese and iron 105 oxides, but this is mere addition and not subtraction from this disclosure. So the H unit or the M. unit, may each embrace several analogous components, provided the members of the H. group or the M. group respectively, 110 have sufficient approximation of fusion points.

For instance, I would not recommend iron and lead oxides as joint components of the M. element, because of the very different 115 fusion points, and because lead tends to globulize when fused with other metals, while tungsten oxide is usable.

It will also be observed that substances 120 usable and classifiable in relation to the H. and M. formula symbols are preferably metallic oxides, usable with such a flux as borax.

The A, B, C, D and E examples I have given as illustration, may be regarded as 125 primary masses, though each in itself is formed of H. M. L. components, that is to say, the H. M. L. material of example A, may constitute the H unit, the H. M. L. material of example B the M. unit, and the H. 130

M. L. material of example E may be the L. unit, selected to constitute the ultimate H. M. L. material or finished product.

Thus the finished product may, on last analysis, comprise quite a variety of different chemical substances, or it may contain only three, but in either event, it conforms to the underlying principle of a resistance material, the specific resistance of which is due 10 to the controllably balanced use of high, medium and low resistance materials, in selected proportions, and the resistance being also predeterminedly influenced by the treatment temperature, or by different pressures, in the instance of formic fabrication.

In the effort to disclose a completely workable basis for utilization of the discovery in the broadest aspect, it is to be understood that I make no claim to scientific accuracy 20 in any theories advanced.

I wish to direct attention to the fact that this present application is intended to be substituted for my pending application, Serial No. 370,282, filed March 31, 1920, which 25 original application will be abandoned in favor of the present case, after it has received filing date and serial number, so as to constitute the present case a continuation of said original.

Having described my invention, I claim: 30 1. The herein described process of forming a resistance element material, consisting in mixing in selected proportions, a very high, a medium and a very low resistance material, and then subjecting them to heat 35 and blending them into a substantially homogeneous composition, then mixing the ma-

terial with different proportions of relatively medium and low resistance materials, and uniting them by ceramic treatments. 40

2. The herein described process of forming an electrical apparatus element product, which consists in first forming by heat treatments a slag-like body containing selected materials of variable electrical resistance, 45 second, reducing the body by attrition, grinding or crushing, and mixing it with predetermined proportions of like materials of variable electrical properties, and third, forming it into a unitary body. 50

3. The herein described process of forming an electrical apparatus heater element, consisting in forming a slag-like body of relatively high, medium and low resistance materials, constituting first, a relatively high 55 resistance material, second, reducing the same and mixing it with materials similar to the original medium and low resistance materials, and third, forming them into a unitary body. 60

4. The herein described process of forming an electrical apparatus element, consisting of forming a slag-like body of materials of variable electrical resistance conforming to the general formula H. M. L. to constitute 65 a H- material, second, reducing the slag and mixing it with variable resistance materials conforming to the general formula H- M. L., and third, forming said mixture into a substantially homogeneous and unitary 70 body.

In witness whereof, I hereunto subscribe my name.

JOHN S. NOWOTNY.